

H. S. FIRMAN, DEC'D.  
W. S. FIRMAN, ADMINISTRATOR.  
PROCESS OF OBTAINING POTASH SALTS FROM SEAWEED.  
APPLICATION FILED FEB. 5, 1910.

1,010,403.

Patented Nov. 28, 1911.



Witnesse: *Lute S. Atch  
Louis W. Gratz*

Henry S. Firman, deceased Inventor  
William S. Firman Administrator  
Revealed your secret at

# UNITED STATES PATENT OFFICE.

HENRY S. FIRMAN, DECEASED, LATE OF SAN DIEGO, CALIFORNIA; WILLIAM S. FIRMAN, ADMINISTRATOR.

## PROCESS OF OBTAINING POTASH SALTS FROM SEAWEED.

1,010,403.

Specification of Letters Patent. Patented Nov. 28, 1911.

Application filed February 5, 1910. Serial No. 542,324.

To all whom it may concern:

Be it known that I, WILLIAM S. FIRMAN, a citizen of the United States, residing at Los Angeles, in the county of Los Angeles and 5 State of California, am the administrator of the estate of HENRY S. FIRMAN, deceased, a citizen of the United States, who resided at San Diego, in the county of San Diego and State of California, and that said 10 HENRY S. FIRMAN did invent a new and useful Process of Obtaining Potash Salts from Seaweed, &c., of which the following is a specification.

This invention is for the purpose of producing potash salts, phosphoric acid, potassic phosphate, etc., by a new and cheap method, from sea-weed or other organic material.

One object of the invention is to produce 20 the potash salt in a coherent dense form especially adapted for commercial purposes, as fertilizer, etc.

The process comprises as essential steps calcination or incineration of the sea-weed, 25 with or without bones or phosphate rock by the combustion of the sea-weed in a suitable chamber or retort, with or without more or less restriction of the air supply according to the result desired. It is preferred to restrict 30 the air supply so that the combustion goes on slowly, and the heat is maintained at a temperature say 700° to 900° F. sufficient for the combustion of the carbonaceous material, but insufficient to cause any substantial loss 35 of the potash salts; the moderate temperature, and the confinement of the material in the chamber during combustion, serving to retain substantially all the potash in the material. When the combustion has been carried 40 to the desired point, the product, while still hot is treated with water or acid solution, or saline solution, as hereinafter described, to cause the product to set into clinker. Sea-weed and other organic ma- 45 terial when treated in this manner yields a product containing a considerable proportion of potassium salts, and also some phosphoric acid, and also some iodin, (iodid and iodate of potassium).

50 In order to increase the percentage of potash ( $K_2O$ ) in the product, it is preferred to use for the wetting down of the hot mass, for the purpose of forming the clinker, as hereinbefore stated, a solution containing potash salts, with or

without other salts or alkali material. This 55 solution may be used at any temperature. It is preferred to use it at a temperature of about 212° F.

The accompanying drawings illustrate an apparatus suitable for carrying out the 60 process.

Figure 1 is a vertical section of the apparatus. Fig. 2 is a plan view of the furnace. Fig. 3 is a horizontal section on the line 65  $x^3-x^4$  Fig. 1.

The furnace comprises a fire box or base 1, formed with the combustion chamber 2, and with fire doors 3 for controlling communication to said combustion chamber from the outside of the furnace, a grate 4 being provided at the bottom of said combustion chamber and supported over an ash pit 6. An upward extension 7 from the combustion chamber 2 is formed preferably with a hollow wall 5 constituting a water jacket in 70 which water or solution may be heated for evaporation or for other purposes connected with the process. A sheet metal tubular body or retort 8 extends upwardly from the chamber 7 and is provided at its upper end 80 with a charging hole 9 having a cover 9', and an outlet 10, said outlet having a valve or damper 11 provided with an operating handle 11'. Ash pit 6 is formed as a runway for a truck 12, for receiving the ash, and is 85 provided with doors 13, for closing the same to the required extent during the burning operation. A tank 14 is provided at any convenient location into which the contents of the truck 12 may be dumped, and means, 90 such as a pipe 15 communicating with the tank or hollow wall 5, may be provided for supplying water to said tank, said pipe preferably having a spray nozzle 16 to spray liquid on to the contents of the tank. Tank 95 5 has charging openings 17.

The process may be used for the production of potash salts, phosphoric acid, potassic phosphate, iodin, iodid and iodate of potassium, etc., from various organic materials, preferably sea-weed in the following manner:—The raw material is first dried, by exposure to the sun and air, or by any suitable method. It is then placed in the upper portion of the furnace through 100 the charging hole. When desired to increase the percentage of phosphoric acid in the product organic or inorganic material is

added, such as bones of commerce, phosphate rock, or any material containing phosphoric acid before or during combustion. When the furnace is filled, the charging hole is closed and the damper is opened. As soon as the fire is well started from the bottom, the damper is nearly closed and the door 13 is also nearly closed so that the admission of air is restricted and the combustion 10 proceeds slowly, with just sufficient heat to gradually consume substantially all or the greater part of the carbonaceous substance in the material undergoing treatment, without sufficient heat to cause material loss of 15 potash by volatilization thereof. When the combustion has reached the desired point, the damper is entirely closed, and one or more fire doors are opened, and the ashes are drawn, raked or dumped into suitable 20 trucks or vehicles and are transported thereby to the dumping station, and there wet down with the water or solution. The truck 12 used for this purpose is preferably run into the ash pit before the burning 25 operation and is inclosed by closing the doors 13, and the grate 4 is preferably a dump-grate, so as to allow the ashes to be quickly dumped into the truck, which is hot by reason of its inclosure within the ash pit, and 30 the ashes are thus delivered to the tank 14 while still retaining the temperature of the furnace, thereby producing most efficient action of the water or concentrating solution in the wetting operation. It is preferred to 35 employ for this purpose water carrying potash salts in solution. The solution may contain other salts in addition to potash salts and may consist of sea-water or saline solution, either natural or produced by lixiviation, or a solution formed from sea-water or 40 saline solution, by evaporation, or concentration, to which sea-water, salt-water, or fresh-water, or other material containing potash or phosphoric acid, or both, may or 45 may not be added before or during concentration or evaporation. The tank or water jacket surrounding the combustion chamber may be conveniently used to heat the water or solution to desired temperature for wetting 50 down the ash for the purpose of obtaining the desired chemical reaction, and for forming the clinker. The saline solution may be produced by lixiviating a portion or batch of the clinker, the resulting solution being used as a concentrating and 55 setting solution for another portion or batch of the clinker.

A suitable solution for the purpose may consist, for example, of potassium chlorid, 60 sodium chlorid, sodium sulfate, and sodium carbonate, dissolved in water. The following may be given as a suitable working range for the solution. KCl 10 to 35, NaCl 30 to 5, Na<sub>2</sub>SO<sub>4</sub> 2 to 8, Na<sub>2</sub>CO<sub>3</sub> 8 to 2, 65 H<sub>2</sub>O 50. The concentration of the fluid

may, however, be varied considerably, say from 20 per cent. to 80 per cent. of water, in place of 50 per cent. as above given.

When the ash has been treated as above described, it is in the form of a hard coherent clinker of great density. This clinker is an article of great value on account of its high potash content. This product is adapted for use in the manufacture of various potash productions, and also for 75 use in the manufacture of fertilizers. Before using it for the above purposes it is preferred to pulverize it. When it is desired to produce certain kinds of fertilizers, more or less phosphoric acid or substances containing phosphoric acid may be added to the clinker, or to the sea-weed before carbonization or before or after pulverization, according to the product or fertilizer desired. 80

In case it is desired to recover iodin 85 from the clinker, this may be done by the usual method of obtaining iodin from ashes containing same.

What I claim is:—

1. The process of producing and concentrating material containing potash from organic substances containing potassium compounds which comprises causing slow combustion of the organic matter in a chamber, while so restricting the admission of air and 90 outflow of products of combustion from the chamber that the temperature is maintained at such a point that substantially all of the potash content of the organic matter is retained in the residue and the greater portion 95 of the carbonaceous content is burned away, and subsequently treating the residue from the combustion with water, while the residue is still sufficiently hot to cause the residue to 100 clinker.

2. The process of producing and concentrating material containing potash from organic substances containing potassium compounds which comprises causing slow combustion of the organic matter in a chamber, 110 while so restricting the admission of air and outflow of products of combustion from the chamber that the temperature is maintained at such a point that substantially all of the potash content of the organic matter is retained in the residue and the greater portion 115 of the carbonaceous content is burned away, and subsequently treating the residue from the combustion with water containing potash salts in solution, while the residue is 120 still sufficiently hot to cause the residue to set to clinker.

3. The process of producing and concentrating material containing potash from organic substances containing potassium compounds which comprises causing slow combustion of the organic matter in a chamber, while so restricting the admission of air and outflow of products of combustion from the chamber that the temperature is maintained 125

- at such a point that substantially all of the potash content of the organic matter is retained in the residue and the greater portion of the carbonaceous content is burned away, and subsequently treating the residue from the combustion with water containing salts of alkali metals including potassium, while the residue is still sufficiently hot to cause the residue to clinker.
- 10 4. The process of producing and concentrating material containing potash and phosphoric acid from sea-weed which consists in causing slow combustion of the sea-weed in a chamber while so restricting the admission of air and outflow of products of combustion from the chamber that the temperature is maintained at such a point that substantially all of the potash content of the sea-weed is retained in the residue and the greater portion of the carbonaceous content is burned away, and subsequently treating the residue from combustion, with water, while the residue is still sufficiently hot to cause the residue to clinker.
- 15 5. The process of producing material containing potash and phosphoric acid from

sea-weed and material containing phosphoric acid, which consists in inclosing in a chamber dry sea-weed together with other material containing phosphoric acid, subjecting the sea-weed and material containing phosphoric acid while so inclosed to slow combustion while so restricting the admission of air and the outflow of the products of combustion that the temperature is maintained at such a point that substantially all of the potash content of the sea-weed is retained in the residue and the greater portion of the carbonaceous content is burned away, and subsequently treating the residue with water, while the residue is still sufficiently hot to cause the residue to clinker.

In testimony whereof, I have hereunto set my hand at Los Angeles, California, this 20th day of January, 1910.

WILLIAM S. FIRMAN,  
*Administrator of the estate of Henry S. Firman, deceased.*

In presence of—

F. M. TOWNSEND,  
THEO. LOHMAN.